

March 31, 1964

F. W. BEALL

3,127,289

METHOD OF DECARBURIZING STEEL COIL

Filed Dec. 4, 1961

2 Sheets-Sheet 1



Fig. 1



Fig. 2



Fig. 3

INVENTOR.  
FRANCIS W. BEALL,  
BY *Young, Blatt, Melville, Rosen*  
ATTORNEYS. *Foster*

March 31, 1964

F. W. BEALL

3,127,289

METHOD OF DECARBURIZING STEEL COIL

Filed Dec. 4, 1961

2 Sheets-Sheet 2



Fig. 4

INVENTOR.  
FRANCIS W. BEALL,

BY  
Youngblut, Merrell, Graessle  
& Fortin  
ATTORNEYS.

# United States Patent Office

3,127,289

Patented Mar. 31, 1964

1

3,127,289

METHOD OF DECARBURIZING STEEL COIL  
Francis W. Beall, deceased, late of Middletown, Ohio, by  
Edythe E. Beall, executrix, Middletown, Ohio, assignor  
to Armco Steel Corporation, Middletown, Ohio, a cor-  
poration of Ohio

Filed Dec. 4, 1961, Ser. No. 157,322

4 Claims. (Cl. 148—16)

The invention relates to the decarburization of steel 10 coil and more particularly to decarburization effected in an opened coil annealing operation.

The decarburizing anneal of steel to remove the strains of cold rolling as well as to remove the carbon from the strip is a known expedient, and hitherto various procedures have been proposed for enhancing the effectiveness of the decarburizing operation. For example, it has been recognized for some time that water vapor is a particularly effective decarburizing substance, and this is particularly true if water vapor is present in controlled amounts in gases containing hydrogen. The atmospheres usually employed are the commercially available and relatively inexpensive gases such as HNX (4-8% H<sub>2</sub>, balance N<sub>2</sub>) or DX (11.5% H<sub>2</sub>, 5% CO<sub>2</sub>, 10% CO, and the balance N<sub>2</sub>). Dissociated ammonia also may be employed. If HNX or DX gas are employed they are normally admixed with sufficient water vapor and hydrogen or dissociated ammonia to establish a dew point in the range of +90° to +130° F. Ideally, the most effective gas is straight hydrogen made as wet as possible while maintaining a non-oxidizing potential; however gas mixtures of various hydrogen contents may be used with suitable dew points to attain comparable results. In any event, in all cases the major decarburization reaction is: C+H<sub>2</sub>O=CO+H<sub>2</sub>, and ideally, the H<sub>2</sub>/H<sub>2</sub>O ratio should be maintained in equilibrium so that the atmosphere in the annealing furnace will be decarburizing and yet non-oxidizing at all times.

Considerable difficulty has heretofore been encountered in endeavoring to maintain the desired equilibrium. As decarburization is effected, some of the water vapor in the incoming gas will be consumed, the consumption varying with the rate of the reaction. If insufficient water vapor is present to offset the quantity consumed, the decarburization process is slowed for want of the decarburizing reactant. On the other hand, if an excessive amount of water vapor is present, the excess moisture will cause scaling which again slows or stops decarburization until the scale is reduced. In addition, such reduced scale is an undesirable contaminant for future processing, such as enameling.

Prior to the instant invention, the customary practice for establishing the desired dew point in the furnace was to maintain the input dew point at a constant level. That is, during the decarburizing portion of the anneal the dew point of the incoming gas was adjusted to the equilibrium level either by admixing water vapor with the gas prior to its introduction into the furnace or by admitting steam along with the gas. However, the difficulty with such prior practice lies in the many variable factors which affect the rate of decarburization and hence the consumption of the water vapor. For example, such factors as the rate at which the carbon in the steel diffuses to the surface where it can react with the water vapor, the rapidity at which the reaction between the carbon and the water vapor takes place, together with the rate at which the moisture laden gas is brought into contact with the surface of the steel, all introduce variables which affect the rate of decarburization. Since ideally, the maximum rate of decarburization will occur under conditions wherein the optimum amount of water vapor is available for reaction no matter how fast or slow the decarburization may be

2

taking place and yet insufficient water vapor is present to cause scaling, the prior art practice of maintaining the input dew point at the equilibrium level does not assure the maintenance of such conditions in the annealing furnace due to the numerous variables which are encountered and which cannot be accurately predicted.

Accordingly, a principal object of the instant invention is the provision of an improved procedure by means of which the H<sub>2</sub>/H<sub>2</sub>O equilibrium of the atmosphere in the furnace is automatically maintained, thereby permitting decarburization to take place at the maximum rate no matter how fast or slow the reaction may be proceeding at any given time during the decarburizing cycle.

A further object of the instant invention contemplates the control of the atmosphere in the annealing furnace during decarburization by maintaining the desired H<sub>2</sub>/H<sub>2</sub>O equilibrium in the exit gas, the hydrogen content and/or the dew point of the incoming gas being varied so as to maintain the desired H<sub>2</sub>/H<sub>2</sub>O equilibrium in the exit gas. In other words, the exit H<sub>2</sub>/H<sub>2</sub>O ratio is maintained constant rather than the input H<sub>2</sub>/H<sub>2</sub>O ratio, as practiced by the prior art.

Still a further object of the instant invention is the provision of a process for decarburizing steel in an annealing furnace in a materially shortened decarburizing cycle utilizing a single control, namely, dew point control of the effluent gas, to maintain essentially optimum decarburizing conditions without scaling. This control is based upon the discovery that, if the exit gas is decarburizing and non-oxidizing, the steel will react accordingly irrespective of inlet gas composition due to the high recirculation rate of the atmosphere and the high rate of the water gas reaction which take place within the furnace.

Still a further object of the instant invention is the provision of decarburization-annealing procedures which may be used in conjunction with any annealing atmosphere gases which are reducing in nature, inclusive of DX gas, HNX gas, hydrogen, or dissociated ammonia, all of which are readily available and inexpensive.

The foregoing, together with other objects of the instant invention which will appear hereinafter or which will be apparent to the skilled worker in the art upon reading this specification, are accomplished by those procedures 45 of which exemplary embodiments shall now be described.

Reference is now made to the accompanying drawings wherein:

FIGURE 1 is a side elevational view with parts broken away and in section of a coil heating furnace.

FIGURE 2 is a graph illustrating a conventional decarburization operation.

FIGURE 3 is a graph similar to FIGURE 2 but illustrating the decarburizing operation of the instant invention.

FIGURE 4 is a graph illustrating the dependence of the H<sub>2</sub>/H<sub>2</sub>O ratio upon furnace temperature.

Referring first to FIGURE 4, the graph plots H<sub>2</sub>/H<sub>2</sub>O equilibria for various annealing temperatures. In order to prevent the steel from oxidizing, the atmosphere within the furnace must lie to the right of the curve, with optimum results being obtained when the H<sub>2</sub>/H<sub>2</sub>O ratio lies on the curve. Thus, where the decarburization portion of the anneal is conducted at a temperature of 1250° F., optimum results will be achieved when the ratio of hydrogen to water vapor is 2.5:1. For a given atmosphere having a known hydrogen content, such equilibrium ratio may be initially established by elevating the dew point of the atmosphere to a predetermined value, which may be on the order of +130° F.

In accordance with prior art practices, and as illustrated by the graph shown in FIGURE 2, the moisture laden atmosphere introduced in the furnace during decarburiza-

tion would be maintained at a constant dew point (+130° F. in the example given) and it will be noted that throughout the decarburizing period the dew point of the effluent gas is substantially below that of the input gas. It will be further noted that the decarburization proceeds at a relatively constant rate—as measured by the carbon monoxide (CO) content of the effluent gas—and that the decarburizing portion of the cycle is on the order of 13 to 14 hours' duration. Since the major decarburization reaction involves the consumption of water vapor and the evolution of hydrogen, the equilibrium condition will be shifted to the right of the curve illustrated in the graph of FIGURE 4, and the decarburization process will be slowed for want of the decarburizing reactant.

In accordance with the instant invention, it has been discovered that the  $H_2/H_2O$  ratio of the exit gas accurately reflects the operating conditions within the furnace, and that by varying the composition of the input gas so as to maintain equilibrium conditions in the effluent gas, the decarburizing operation can be conducted with maximum efficiency and in a greatly reduced time. Thus, by varying the input dew point and/or input hydrogen, it is possible to control the ratio of the exit gas to maintain an essentially constant reducing potential at substantially equilibrium conditions. It is believed that the input gas does not contact the surfaces of the coils being treated until it has been diluted and reacted by the gases already present in the furnace. Thus the exit gas is believed to be indicative of the average composition of the gases in the furnace and hence an accurate indicator of the  $H_2/H_2O$  ratio.

It is thus possible, by measuring both the dew point and the hydrogen content of the effluent gas, to vary the relative amounts of hydrogen and water vapor in the input gas, so as to thereby maintain equilibrium conditions in the effluent gas. However, such controls are relatively complex due to the number of variables which must be calibrated. Consequently, while it is possible to control the  $H_2/H_2O$  ratio of the effluent gases, it has also been discovered that the desired equilibrium conditions can be closely approached solely by varying the input dew point so as to maintain a constant dew point in the effluent gas at the equilibrium level for the gas employed. Where this is done, a materially enhanced rate of decarburization is obtained. Thus, in accordance with a preferred embodiment of the instant invention, and as exemplified by the graph of FIGURE 3 wherein the exit dew point of the gas is maintained at a constant value of +130° F. throughout the decarburizing portion of the cycle, it will be seen that the rate of decarburization—again as measured by the quantity of carbon monoxide in the effluent gas—is far more rapid, the entire decarburizing portion of the annealing cycle taking place in between 8 and 9 hours, as compared to the 13 to 14 hours required in the example of FIGURE 2. As indicated by the dotted line in FIGURE 3, the input dew point of the atmosphere rises appreciably during the initial stage of the decarburizing cycle; but it is at all times sufficient to maintain the dew point of the effluent gas at the desired constant level. Essentially, the peak value of the input dew point is a function of the peak decarburization rate and varies with the amount of carbon being removed. However, a typical peak value for input dew point would be +160° F. when controlling the exit dew point at +130° F.

Essentially, the instant invention may be practiced in conjunction with known decarburizing and annealing techniques. Thus, the operation begins by the open winding of the steel strip into coils. Such open or loose winding contemplates the insertion of a spacer, which may comprise string, a metal tape, or a twisted wire, between each convolution of the coil. This produces a uniform space between each convolution, thereby permitting free passage of the gas between the convolutions and hence all over contact of the gas with the entire surface areas of

the loose coiled strip. Commercial coiling units are available for this purpose.

Subsequent to the formation of the opened coil, it is transferred to the annealing base of an annealing furnace such as a Lee Wilson furnace, whereupon the covers are set in place and the furnace readied for the decarburizing and annealing operation. Such furnace is diagrammatically illustrated in FIGURE 1 wherein the opened coils 1 are seated on the base assembly 2 and surrounded by 10 the inner cover 3 which is preferably sealed to the base assembly to render it completely gas tight. The outer cover or furnace is indicated at 4, the furnace being provided with suitable heating means 5. A gas inlet is provided at 6 for introducing the desired atmosphere within 15 the inner cover 3; and a gas outlet is provided at 7. A fan 8 acts to rapidly recirculate the atmosphere within the furnace and cause it to pass between the convolutions of the coils. In normal use, a dry atmosphere, at a dew point of say —40° F., will be introduced into the furnace 20 while the furnace is brought to temperature, whereupon the dew point of the atmosphere will be elevated to the desired level for the decarburizing portion of the cycle.

In accordance with the preferred embodiment of the invention, the moisture content of the effluent gas is 25 measured by a dew meter 9, such as a Foxboro Dewcel, operatively connected to the gas outlet 7 and acting to measure the moisture content of the effluent gas; and the dew meter is connected to a recording controller 10 which is in turn connected to the control valve 11 by means of 30 which steam is introduced through pipe 12 into the gas inlet 6. With this arrangement, the control valve 11 will be opened and closed in such fashion that additional steam will be injected into the incoming gas as the moisture content of the effluent gas drops below the predetermined level; and similarly, should the dew point of the effluent gas rise above the desired level, the dew meter will 35 act to reduce or shut off the steam flow until the desired effluent dew point has been reestablished.

The end of the decarburization period is determined 40 by measuring the carbon monoxide (CO) content of the effluent gas and, when the decarburizing reaction product reaches a predetermined low value (about 1% or less), dry gas may be again injected into the furnace for the cool-down period. It will be understood that any 45 CO in the input gas must be considered in determining the end point. In this connection, it is to be understood that the control of the atmosphere in the annealing furnace both prior to and subsequent to the decarburizing portion of the annealing cycle does not constitute a limitation on the instant invention; and known annealing techniques may be employed.

As should now be apparent, the instant procedure provides for a materially enhanced rate of decarburization through the use of a constantly controlled annealing atmosphere dew point. In other words, one of the 55 reactants, namely, water vapor, is supplied at a rate equal to its consumption and demand in the decarburizing reaction. In addition to increasing productivity, the constant control of the exit dew point acts to prevent oxidation of the metal. Yet it has been found that exceedingly high initial input dew points, i.e. substantially in 60 excess of the desired equilibrium dew point, do not result in scaling of the strip provided the dew point of the effluent gas does not exceed the equilibrium conditions. 65 As has been pointed out, it is believed that the desired equilibrium conditions are achieved in the furnace irrespective of the presence of excessive amounts of water vapor in the incoming gas by reason of the rapid recirculation of the gas and its dilution and reaction with the relatively dry gas already present in the furnace.

The instant procedure contemplates the use of any annealing atmosphere gases which are reducing in nature, such as the aforementioned DX, HNX, dissociated ammonia or hydrogen gases and mixtures of the same. The maximum effluent gas dew point is limited only by the

$H_2/H_2O$  equilibrium at the desired annealing temperature in order to prevent scaling. As a practical matter, the maximum useful dew point will be about +160° F. and the minimum useful dew point will be about +70° F. The desired annealing temperature will be determined by the type of steel being treated; but in general the temperature range will be from about 1100° to 1500° F. By and large, it is preferred to decarburize at a temperature of about 1250° to 1350° F. Hydrogen may be added to the common bright annealing gases during the soak period of the annealing cycle in order to increase the allowable dew point, thereby further increasing the decarburizing efficiency.

Having thus described the invention in certain exemplary embodiments, and with the understanding that modifications may be made therein without departing from its spirit and purpose, what is desired to secure and protect by Letters Patent is:

1. The method of controlling the hydrogen/water vapor volume ratio of a hydrogen containing reducing atmosphere in an annealing furnace during the decarburization of steel coil, which method comprises maintaining the atmosphere in the furnace at a temperature of from about 1100° F. to 1500° F. during decarburization, and varying the dew point of the atmosphere as it is introduced into the furnace to the extent necessary to maintain the dew point of the effluent atmosphere at an essentially constant level, at which level the hydrogen/water vapor volume ratio of the effluent atmosphere is within the range of 2.0:1 to 3.5:1, the hydrogen/water vapor volume ratio at any given temperature being so chosen that the effluent atmosphere is at all times decarburizing and non-oxidizing to the steel coil being treated.

2. The method claimed in claim 1 wherein the dew point of the effluent atmosphere is maintained at the said

essentially constant level until the carbon monoxide content of the effluent atmosphere due to the major decarburization reaction  $C+H_2O=CO+H_2$  has fallen below a value on the order of about one percent.

5 3. A method of decarburizing steel coil in a continuously circulating hydrogen containing reducing atmosphere having a controlled hydrogen/water vapor volume ratio, which method comprises maintaining the circulating atmosphere in the furnace at a temperature of from about 1100° F. to 1500° F. during decarburization, and maintaining the hydrogen/water vapor volume ratio of the effluent atmosphere at an essentially constant level by varying the quantity of moisture introduced into the entering atmosphere, the quantity of moisture introduced into the entering atmosphere being the amount necessary to maintain the dew point of the effluent atmosphere at from about +70° F. to about +160° F., the dew point at any given temperature being so chosen that the effluent atmosphere is at all times decarburizing and non-oxidizing to the steel coil being treated.

10 4. The method claimed in claim 3 wherein the dew point of the effluent atmosphere is maintained at the chosen essentially constant level until the carbon monoxide content of the effluent atmosphere due to the major decarburization reaction  $C+H_2O=CO+H_2$  has fallen below a value on the order of about one percent.

#### References Cited in the file of this patent

##### UNITED STATES PATENTS

|              |                        |               |
|--------------|------------------------|---------------|
| 30 2,287,467 | Carpenter et al. ----- | June 23, 1942 |
| 2,557,379    | Hancock et al. -----   | June 19, 1951 |
| 2,753,170    | Ness et al. -----      | July 3, 1956  |
| 3,021,237    | Henke -----            | Feb. 13, 1962 |
| 35 3,030,240 | Crombie et al. -----   | Apr. 17, 1962 |